

## UNITED STATES PATENT OFFICE

JOSEPH FRANCIS KING, OF PORTLAND, MAINE, ASSIGNOR OF ONE-FOURTH TO THOMAS M. DONAHUE AND ONE-FOURTH TO JOHN E. DONAHUE, BOTH OF PORTLAND, MAINE

## COMPOSITION FOR TREATING PULP

No Drawing.

Application filed January 28, 1931. Serial No. 511,931.

This invention relates to a process and composition for treating pulp made from grass and wood. Fahr. for approximately four hours, after which the pulp is washed and dried.

An object of the invention is the provision of a composition for treating pulp to give to the pulp a dull finish so that when the same is manufactured into rayon a dull tone or subdued finish will be provided which will be retained when the pulp has been manufactured into rayon.

A further object of the invention is the provision of a process for bleaching, weighting, softening, for giving a dull finish to pulp which is to be manufactured into rayon with the subdued finish being retained in the manufactured rayon, the process requiring considerably less time to complete the finished product than has been done formerly while giving to the product a dull tone which is retained when materials are manufactured into rayon.

This invention will be best understood from a consideration of the following detailed description; nevertheless, it is to be understood that the invention is not confined to the disclosure, being susceptible of such changes and modifications which shall define no material departure from the salient features of the invention as expressed in the appended claims.

In carrying out my invention I have provided a process which will clean, soften, bleach and give a dull finish to sulphite pulp and paper in all stages.

For every hundred pounds of pulp I employ a composition consisting of approximately four parts by weight of sodium perborate, one part by weight of magnesium carbonate, one part by weight of Epsom salts or magnesium sulphate in crystallized form, one-half part of cocoanut oil soap, one part by weight of sodium hyposulphite, one-half part of barley malt paste and one-half part by weight of sodium bisulphite. In other words for every hundred pounds of pulp eight and one-half pounds of the above composition is used. The sulphite pulp is placed in a kier or vat and the ingredients of the composition are dissolved in boiling water and the whole is maintained at 180°

An important feature of the invention resides in the fact that a dull finish or subdued tone is given to the pulp which is retained after the same has been manufactured into rayon and this dull tone is obtained by the use of magnesium carbonate. The sodium perborate acts as a bleaching agent while the sodium hyposulphite gives weight to the material and also acts as a binder.

The cocoanut oil soap produces a softening effect upon the material while the barley malt acts as a cleaner for removing gums, oils, and other resinous matter from the pulp.

Due to the fact that the sodium bisulphite is slightly acid in re-action it aids in maintaining the acid condition of the materials in the kier.

It will be seen from the above that a product is produced which has a subdued finish or dull tone which is free from foreign matter such as resinous materials, has a soft texture and has the proper weight suitable for the purpose.

I claim:

1. A composition of the class described comprising sodium perborate, magnesium carbonate, crystals of magnesium sulphate, cocoanut oil soap, sodium hyposulphite, barley malt and sodium bisulphite.

2. A composition of the class described comprising four parts by weight of sodium perborate, one part by weight of magnesium carbonate, one part by weight of magnesium sulphate, one-half part by weight of cocoanut oil soap, one-half part by weight of sodium hyposulphite, one-half part by weight of barley malt and one-half part by weight of sodium bisulphite.

3. A composition of the class described comprising a bleaching agent, an agent for removing resinous materials, a softening agent, and carbonate of magnesium.

JOSEPH FRANCIS KING.